

Sept. 1, 1953

R. ADLER

2,650,999

CATHODE STRUCTURE FOR ELECTRON-DISCHARGE DEVICES

Filed April 11, 1950



ROBERT ADLER  
INVENTOR.

BY *Francis W. Coffey*  
HIS ATTORNEY

## UNITED STATES PATENT OFFICE

2,650,999

CATHODE STRUCTURE FOR ELECTRON-  
DISCHARGE DEVICESRobert Adler, Northfield, Ill., assignor to Zenith  
Radio Corporation, a corporation of Illinois

Application April 11, 1950, Serial No. 155,208

10 Claims. (Cl. 313—302)

**1**

This invention relates to electron-discharge devices and more particularly to improved electrodes or other elements for incorporation in such devices.

In the processing of a thermionic oxide-coated cathode, it is conventional practice to coat a conductive sleeve with carbonates of barium, strontium, calcium, and/or similar metals and subsequently to subject the coated cathode sleeve to intense heat (usually 900° C. or higher) in order to decompose the carbonates into the corresponding oxides and to drive off carbon dioxide gas. This operation is generally performed while the device is connected to a vacuum pump so that the carbon dioxide gas which is driven off as a result of decomposition of the carbonates is evacuated from the tube; consequently, the operation is conventionally referred to as the "outgassing" operation. In subsequent processing, the tube may be completely evacuated and gettered in a conventional fashion, and the oxide-coated cathode so formed may be seasoned in a well-known manner until such time as full electron-emissivity is obtained.

By far the greatest number of high-vacuum oxide-cathode electron tubes produced at the present time comprise internal resistance elements associated with the cathode sleeve for energizing the cathode during operation of the tube. Internal heater elements of this type furnish a very convenient means for elevating the temperature of the carbonate-coated cathode sleeve to a sufficient extent to provide complete outgassing of the carbonates. Thus, in outgassing tubes of this type, the internal indirect-heater element is provided with sufficient current to raise the temperature of the cathode sleeve high enough to satisfy the outgassing requirements.

There are other high-vacuum electron-discharge tubes known to the art, however, which comprise indirectly-heated thermionic cathodes not provided with internal heater resistance elements. For example, there is disclosed and claimed in the copending application of Robert Adler, Serial No. 129,554, filed November 26, 1949, for "Electron-Discharge Devices and Circuits," and assigned to the present assignee, a novel electron-discharge device having a bi-directional electron-discharge path. Briefly, such a bilaterally conductive device comprises a pair of thermionic cathodes disposed at opposite ends of a common electron-discharge path; a control grid is provided between the cathodes for controlling the conductivity of the device. In its

**2**

preferred application as a switch tube in a saw-tooth current generator, voltage pulses of large amplitude are produced between the cathodes. Consequently, in order to avoid the necessity for providing special high-voltage insulation, it is preferred that one of the cathodes be energized in operation by means other than a conventional internal resistance heater element. For example, a preferred construction of such a tube may comprise a bipartite outer cathode and a second or inner cathode disposed between the component parts of the outer cathode and substantially surrounded by a control grid. Each part of the outer cathode may be provided with an associated resistance element for heating, while the inner cathode is not provided with such an energizing element but instead is adapted to be energized in operation partly by radiant heat from the outer cathode and partly by heat developed by plate dissipation at the inner cathode in its role as anode during the portion of each cycle in which it operates at a higher potential than the outer cathode.

Since the inner cathode of a switch tube of the type discussed is not provided with an associated internal heater resistance element, some other means must be employed to elevate the temperature of the inner cathode during the processing of the tube in order to provide complete outgassing of the carbonates. It is not feasible to heat the inner cathode during the outgassing operation by electron bombardment from the outer cathode because this has been found to be too destructive of the thermionic coating. Moreover, raising the temperature of the inner cathode to an extent sufficient to provide complete outgassing of the carbonates by induction heating by eddy current loss has been found to have detrimental effects, such as warpage and the like, upon the control grid surrounding the inner cathode. It is therefore apparent that conventional outgassing methods are not practical for use in the processing of a switch tube of the type under consideration.

It is an important object of the present invention to provide a new and improved element for an electron-discharge device. It is a further object of the invention to provide an improved electrode for an electron tube. Yet another object of the invention is to provide a new and improved thermionic cathode.

Still another object of the invention is to provide a bilaterally conductive switch tube of the type disclosed in the above-identified Adler application comprising a new and improved inner

cathode which may be readily processed without undesirably affecting the other tube elements.

In accordance with the present invention, as specifically applied to a switch tube of the type discussed above, the inner cathode is constructed at least in part of a ferromagnetic material having a Curie point higher than that of iron. Preferably, the ferromagnetic material used is a ferro-cobalt or a nickel-cobalt alloy, and the Curie point of the alloy selected is preferably above 900° C. However, in its broader aspects, the invention also contemplates the use of such a ferromagnetic material in the construction of any electrode or other element having a solid cross-section in a high-vacuum electron-discharge device.

The features of the present invention which are believed to be novel are set forth with particularity in the appended claims. The invention, together with further objects and advantages thereof, may best be understood, however, by reference to the following description considered in conjunction with the accompanying drawing, in which the single figure is a cross-sectional view of an electron-discharge device comprising a thermionic cathode constructed in accordance with the present invention.

In the drawing, a bilaterally conductive electron-discharge device comprises a plurality of elements supported within an evacuated envelope 10 in any convenient manner well-known to the art. The device comprises a bipartite outer cathode, consisting of two component parts 11 and 12 respectively provided with oppositely disposed electron-emissive coatings 13 and 14. A second or inner cathode 15 is disposed between parts 11 and 12 of the bipartite outer cathode and is substantially surrounded by a control grid 16 which may conveniently be constructed as a helical winding about a pair of side-rods or supporting posts 17 and 18, although the specific construction of the control grid is not material to the present invention. Component parts 11 and 12 of the outer cathode are individually provided with heater resistance elements 19 and 20 insulatedly supported internally of the respective composite parts 11 and 12, and a pair of heat shield members 21 and 22 are arranged to reflect radiant heat from the outer cathode inwardly in order to energize the inner cathode 15 during operation of the tube. Heat-radiating fins 23 and 24 are affixed respectively to grid side-rods 17 and 18 to prevent over-heating of the grid wires. To this end, the outer surfaces of radiating fins 23 and 24 are preferably blackened to provide efficient heat radiation, while the inner surfaces are highly polished to prevent substantial radiation inwardly toward the central structure.

The inner cathode 15 may conveniently be constructed by forming a pair of thermionically emissive coatings 25 and 26 on opposite surfaces of a suitable cathode sleeve member 27. No internal heater resistance element is provided for inner cathode sleeve member 27; rather, in accordance with the invention, a ferromagnetic slug or insert 28 is disposed within cathode sleeve 27. Insert 28 is constructed of a ferromagnetic material having a Curie point higher than that of iron (about 760° C.) and preferably above 900° C. Suitable materials for this purpose include certain ferro-cobalt alloys, and a ferro-cobalt alloy having a cobalt content of from 30% to 50% by weight is preferred. Small amounts of

vanadium, chromium, or other metals may be incorporated in the alloys to provide ductility and other desirable metallurgical properties. One material which has been found particularly suitable is a ferro-cobalt alloy having a cobalt content of substantially 35% and including about 1½% or 2% vanadium; this material is commercially available under the trade names "Perendur" and "Hiperco" and has a Curie point of about 950° C. Nickel-cobalt alloys having a cobalt content greater than 40% by weight also have Curie points higher than that of iron and hence are suitable for the purposes of the invention. Pure cobalt is ferromagnetic and has a Curie point of about 1130° C. and is therefore also suitable for use in accordance with the invention; however, pure cobalt is very difficult to work, in a metallurgical sense, so that ferro-cobalt or nickel-cobalt alloys having somewhat lower Curie points but having more desirable metallurgical properties are preferred.

As an alternative, it is apparent that the inner cathode 15 may be formed with the ferromagnetic insert 28 as a base member. Thus, member 28 may be provided with a nickel plating or the like to which thermionically emissive coatings 25 and 26 may readily adhere. In any event, ferromagnetic member 28 may be viewed as a structural part of the inner cathode 15.

In the processing of the illustrated device, the inner cathode sleeve member 27 is provided with suitable carbonate coatings in a manner well known in the art, and the tube elements are placed within envelope 10. The tube is then connected to a vacuum pump or evacuating device (not shown). Outgassing of the carbonate coatings on the inner cathode sleeve member 27 is readily accomplished by providing an electromagnetic induction heating field in a direction perpendicular to the plane of the drawing; any conventional induction heating apparatus (not shown) may be used for this purpose, one particularly suitable device comprising a helical coil which may be disposed coaxially about tube envelope 10 and which is driven from a suitable high-powered source to provide the desired field intensity.

The provision of an axial heating field results in a rapid increase in the temperature of ferromagnetic insert 28, due to the hysteresis loss of the material. As the temperature of the insert 28 approaches the Curie point, the hysteresis loop shrinks, so that the energy dissipation per cycle due to hysteresis loss decreases. At temperatures above the Curie point, the material behaves substantially like any paramagnetic material; in other words, at such temperatures there is no energy dissipation due to hysteresis loss. Because the direction of the induction heating field is substantially parallel to the flat surfaces of the inner cathode, the amount of eddy current heating in the ferromagnetic insert 28 is so small as to be practically negligible. Consequently, the ferromagnetic insert behaves substantially as its own thermostat, rising to a temperature near its Curie point in response to an applied axial induction heating field and maintaining its temperature near the Curie point so long as the field is of sufficient intensity.

Heating of the inner cathode during the outgassing operation by hysteresis loss is preferred over eddy current heating for the reason that control grid 16 is also elevated in temperature by eddy current loss in the grid structure. For a given flux density, hysteresis loss is proportional

to the frequency of the induction heating field, while eddy current loss is proportional to the square of the frequency. Thus, by maintaining the frequency of the heating field at a relatively low value (but high enough that heat is produced at the rate required), and by constructing the control grid of non-magnetic or paramagnetic material, a high flux density may be used without over-heating control grid 16. A frequency of the order of 1 megacycle has been found quite acceptable in practice.

Thus, the present invention provides an improved thermionic cathode of the heaterless variety which may, for example, be advantageously incorporated in a bi-directional electron-discharge device of the type disclosed and claimed in the above-identified Adler application. Although the invention affords exceptional advantage in this environment, it is also contemplated that other solid electrodes or elements of the internal structure of this or of other types of electron-discharge device may be constructed of a ferromagnetic material having a Curie point higher than that of iron, in order to facilitate heating such electrode or element by an induction heating field, in accordance with the invention. For example, it may be desirable in some instances to construct grids, anodes, or other cold electrodes of such material, in order that such electrodes may readily be freed of occluded gases during the processing of the tube.

While a particular embodiment of the present invention has been shown and described, it is apparent that various changes and modifications may be made, and it is therefore contemplated in the appended claims to cover all such changes and modifications as fall within the true spirit and scope of the invention.

I claim:

1. An electron-discharge device element having a solid cross-section and constructed at least in part of a ferromagnetic material having a Curie point higher than that of iron.

2. An electron-discharge device electrode having a solid cross-section and constructed at least in part of a ferromagnetic material having a Curie point higher than that of iron.

3. An electron-discharge device element having a solid cross-section and constructed at least in part of a cobalt alloy having a Curie point higher than that of iron.

4. An electron-discharge device element having a solid cross-section and constructed at least in part of a ferro-cobalt alloy having a Curie point higher than that of iron.

5. An electron-discharge device element having a solid cross-section and constructed at least in part of a ferro-cobalt alloy having a cobalt content of from 30% to 50% by weight and having a Curie point above 900° C.

10 6. An electron-discharge device element constructed at least in part of a nickel-cobalt alloy, the cobalt comprising more than 40% by weight of the alloy, said alloy having a Curie point higher than that of iron.

15 7. An electron-discharge device element constructed of substantially pure cobalt.

8. A thermionic cathode comprising: a hollow sleeve; a thermionically emissive coating on at least one surface of said sleeve; and a ferromagnetic insert for said sleeve having a solid cross-section and constructed of a material having a Curie point higher than that of iron.

20 9. An electron-discharge device comprising: a bipartite thermionic cathode; indirect-heater means for said bipartite cathode; and a heaterless thermionic cathode, disposed between the composite parts of said first-mentioned cathode and substantially surrounded by a control grid, constructed at least in part of a ferromagnetic material having a Curie point higher than that of iron.

25 10. An electron-discharge device comprising: a bipartite thermionic cathode; indirect-heater means for said bipartite cathode; and a heaterless thermionic cathode, disposed between the composite parts of said first-mentioned cathode and substantially surrounded by a control grid, constructed at least in part of a ferro-cobalt alloy having a cobalt content of from 30% to 50% by weight and having a Curie point above 900° C.

ROBERT ADLER.

References Cited in the file of this patent

UNITED STATES PATENTS

| Number    | Name    | Date          |
|-----------|---------|---------------|
| 1,931,737 | Parisi  | Oct. 24, 1933 |
| 2,140,534 | Mahoney | Dec. 20, 1938 |
| 2,192,491 | Widell  | Mar. 5, 1940  |
| 2,410,822 | Kenyon  | Nov. 12, 1946 |